



US006415638B1

(12) **United States Patent**  
Sakurai et al.

(10) Patent No.: US 6,415,638 B1  
(45) Date of Patent: Jul. 9, 2002

- (54) **METHOD AND DEVICE FOR FORMING TUBULAR WORK INTO SHAPED HOLLOW PRODUCT BY USING TUBULAR HYDROFORMING**

JP 63-220929 \* 9/1988 ..... 72/58

## OTHER PUBLICATIONS

- (75) Inventors: **Hiroshi Sakurai**, Tokyo; **Eizaburo Nakanishi**; **Shinji Ooe**, both of Yokohama; **Masanobu Hayasaka**; **Junji Katamura**, both of Kanagawa, all of (JP)

(73) Assignee: **Nissan Motor Co., Ltd.**, Yokohama  
(JP)

(\*) Notice: Subject to any disclaimer, the term of this patent is extended or adjusted under 35 U.S.C. 154(b) by 0 days.

(21) Appl. No.: 09/534,261

(22) Filed: Mar. 24, 2000

(30) **Foreign Application Priority Data**

|                          |             |
|--------------------------|-------------|
| Mar. 26, 1999 (JP) ..... | 11-083658   |
| Jun. 29, 1999 (JP) ..... | 11-183920   |
| Dec. 24, 1999 (JP) ..... | 11-366894   |
| Feb. 25, 2000 (JP) ..... | 2000-049476 |

(51) Int. Cl.<sup>7</sup> ..... B21D 26/02

(52) U.S. Cl. .... 72/57; 72/55; 72/58

(58) **Field of Search** ..... 72/55, 57, 58,  
..... 72/61, 62

(56) **References Cited**

## U.S. PATENT DOCUMENTS

|           |    |   |         |                     |        |
|-----------|----|---|---------|---------------------|--------|
| 4,829,803 | A  | * | 5/1989  | Cudini .....        | 72/367 |
| 5,339,667 | A  | * | 8/1994  | Shah et al. .....   | 72/58  |
| 5,974,846 | A  | * | 11/1999 | Ash .....           | 72/55  |
| 6,237,382 | B1 | * | 5/2001  | Kojima et al. ..... | 72/58  |
| 6,257,035 | B1 | * | 7/2001  | Marks et al. .....  | 72/57  |

## FOREIGN PATENT DOCUMENTS

JP 61-186127 \* 8/1986 ..... 72/58

**30 Claims, 22 Drawing Sheets**



**FIG.1****FIG.2**

**FIG.3**



**FIG. 4**



**FIG.5****FIG.6**

**FIG.7****FIG.8**

## FIG.9



**FIG.10****FIG.11**

**FIG.12**



**FIG.13**



**FIG.14**

FIG.15



FIG.16



FIG.17



FIG.18



**FIG.19**

**FIG.20****FIG.21**

**FIG.22****FIG.23**

**FIG.24****FIG.25**

**FIG.26****FIG.27**

**FIG.28****FIG.29**

**FIG.30****FIG.31**

**FIG.32****FIG.33**

**FIG.34****FIG.35**

**FIG.36**

FIG.37



**METHOD AND DEVICE FOR FORMING  
TUBULAR WORK INTO SHAPED HOLLOW  
PRODUCT BY USING TUBULAR  
HYDROFORMING**

**BACKGROUND OF THE INVENTION**

**1. Field of the Invention**

The present invention relates in general to tubular hydroforming and more particularly to method and device for forming a tubular work into a shaped hollow product by using hydroforming process. More specifically, the present invention relates to method and device for producing an automotive hollow part, such as front pillar, center pillar, roof rail or the like, by using tubular hydroforming process.

**2. Description of the Prior Art**

Tubular hydroforming process is a novel process that has recently gained much attention due to its cost-effective application particularly in the automotive industry. As is known, the tubular hydroforming is of a process that includes major steps wherein ends of a tubular work in a net shape die unit are sealed and a hydraulic fluid is pumped in the tubular work and pressurized to deform cross-sections of the work to conform to a cross section of the net shape die. Usually, before the major steps, a pre-forming is made wherein for obtaining a pre-defined shape of the tube that closely resembles the final component (viz., hollow product), a die closing is gradually carried out while receiving a relatively low hydraulic fluid in the work. While, in a so-called bulging process in the tubular hydroforming, axial feed is provided along the longitudinal axis of the tubular work in the net shape die while receiving the hydraulic fluid in the work. When employing this bulging process, a tube wall thinning during the hydroforming process can be reduced.

However, due to the nature of deformation of the material of the tubular work during the hydroforming process, it has been difficult to provide a hydroformed hollow product that gives users satisfaction. In fact, in the pre-forming step, even when aluminum and/or high strength steel tube is used as the tubular work, a crack tends to appear at a portion that has been subjected to a wall thinning during the expansion of the work. Furthermore, in the pre-forming step, a corner portion remote from the center of the work is particularly attacked by such wall thinning. In the bulging process, wall thickening throughout the length of the tubular work is readily made, however wall thickening at a specified or needed portion, such as a corner portion or the like, is not readily made, and thus, reduction in weight of the hydroformed hollow product has not been satisfactorily achieved particularly in the field of automotive industry.

**SUMMARY OF THE INVENTION**

It is therefore an object of the present invention to provide a method for forming a tubular work into a shaped hollow product by using hydroforming process, which method is free of the above-mentioned drawbacks.

It is further an object of the present invention to provide a hydroforming device which is suitable for practically carrying out the method of the present invention.

It is further an object of the present invention to provide a hydroforming method by which a specified or needed portion of a shaped hollow product can be exclusively thickened.

According to the present invention, there is provided a method for forming a tubular work into a shaped hollow

product by using hydroforming process. In the method, female and male dies are prepared. The female die has a longitudinally extending cavity which has a polygonal cross section when receiving the male die. The tubular work is placed into the cavity of the female die. The interior of the tubular work is then fed with a hydraulic fluid, and the pressure of the fluid is increased to a given level. The given level is smaller than a critical level that causes a bulging of the tubular work. The male die is then pressed against the tubular work to deform the same while keeping the hydraulic fluid at the given level, thereby forming a shaped hollow product that has a polygonal cross section that conforms to that of the cavity. The pressing work is continued until a circumferential length of the shaped hollow product becomes shorter than that of the tubular work.

According to the present invention, there is further provided a hydroforming device for forming a tubular work into a shaped hollow product by using a hydroforming process. The device comprises a fixed female die having a longitudinally extending cavity, the cavity being sized to receive therein the tubular work; a male die having a work surface, the male die being movably received in the female die in such a manner that the work surface of the male die faces the cavity to cause the cavity to be enclosed and have a polygonal cross section; at least one projection formed on a lateral end of the work surface, the projection having a sloped surface angled relative to the work surface and an actuator which actuates the male die to press against the tubular work.

**BRIEF DESCRIPTION OF THE DRAWINGS**

FIG. 1 is a longitudinally sectional view of a hydroforming device used for practically carrying out a method of a first embodiment of the present invention;

FIG. 2 is a view similar to FIG. 1, but showing a different or pressing condition of the device;

FIG. 3 is a perspective view of the hydroforming device for carrying out the method of the first embodiment;

FIG. 4 is a schematically illustrated laterally sectional view of the hydroforming device of FIG. 3;

FIG. 5 is a sectional view of a shaped hollow product provided by the method of the first embodiment;

FIG. 6 is a schematic illustration showing a test for examining a mechanical strength of the shaped hollow product;

FIG. 7 is a graph showing the results of the test;

FIG. 8 is a graph showing results of other test;

FIG. 9 is a schematically illustrated female die used in a hydroforming device which is used for carrying out a method of a second embodiment of the present invention;

FIG. 10 is a partial sectional view of a female die used in a hydroforming device which is used for carrying out a method of a third embodiment of the present invention;

FIG. 11 is a graph showing results of a test for finding a desired angle of an extra slanted wall possessed by the female die of FIG. 10;

FIG. 12 is a longitudinally sectional view of a hydroforming device used for carrying out a method of a fourth embodiment of the present invention;

FIG. 13 is a view similar to FIG. 12, but showing a different or pressing condition of the device;

FIG. 14 is a sectional view of a shaped hollow produced provided by the method of the fourth embodiment;

FIG. 15 is a laterally sectional view of a hydroforming device used for carrying out a method of a fifth embodiment of the present invention;

FIG. 16 is a graph showing results of a test for examining the thickness increasing rate relative to male die pressing stroke;

FIG. 17 is a laterally sectional view of a hydroforming device used for carrying out a method of a sixth embodiment of the present invention;

FIG. 18 is a laterally sectional view of a hydroforming device used for carrying out a method of a seventh embodiment of the present invention;

FIG. 19 is a laterally sectional view of a hydroforming device used for carrying out a method of an eighth embodiment of the present invention;

FIG. 20 is a laterally sectional view of a hydroforming device used for carrying out a method of a ninth embodiment of the present invention;

FIG. 21 is a sectional view of a shaped hollow product provided by the method of the ninth embodiment;

FIG. 22 is a laterally sectional view of a hydroforming device used for carrying out a method of a tenth embodiment of the present invention;

FIG. 23 is a sectional view of a shaped hollow product provided by the method of the tenth embodiment;

FIG. 24 is a laterally sectional view of a reference hydroforming device which was used for proving improvement achieved by the tenth embodiment of the invention;

FIG. 25 is a sectional view of a shaped hollow product provided by the device of FIG. 24;

FIG. 26 is a laterally sectional view of a hydroforming device used for carrying out a method of an eleventh embodiment of the present invention;

FIG. 27 is a sectional view of a shaped hollow product provided by the method of the eleventh embodiment;

FIG. 28 is an enlarged sectional view of one of four corner portions of the shaped hollow product shown in FIG. 27;

FIG. 29 is a graph showing results of a measurement for measuring the thickness of various positions of the corner portion;

FIG. 30 is a laterally sectional view of a hydroforming device used for carrying out a method of a twelfth embodiment of the present invention;

FIG. 31 is an enlarged view of a part of the device of FIG. 30, showing a pressing condition of the device;

FIG. 32 is a sectional view of a shaped hollow product provided by the method of the twelfth embodiment;

FIG. 33 is an enlarged sectional view of one of four projected round corner portions of the product of FIG. 32;

FIG. 34 is a laterally sectional view of a reference hydroforming device which was used for proving improvement achieved by the method of the twelfth embodiment;

FIG. 35 is an enlarged view of a part of the device of FIG. 34, showing a pressing condition of the device;

FIG. 36 is a graph showing results of a measurement for measuring the thickness of various portions of the projected round corner portion of the product of FIG. 32; and

FIG. 37 is a perspective view of an automotive body and frame construction having front pillars, center pillars, side roof rails and the like which can be provided by tubular hydroforming process.

#### DETAILED DESCRIPTION OF THE EMBODIMENTS

In the following, the present invention will be described in detail with reference to the drawings.

For ease of understanding, directional terms, such as upper, lower, right, left, vertical, horizontal, upward, downward, and the like are used in the description. However, it is to be noted that such terms are to be understood with respect to only a drawing or drawings on which the corresponding parts or structures are illustrated.

Referring to FIGS. 1 to 8, particularly FIGS. 1 to 4, there is shown a hydroforming device 1 with which a method of a first embodiment of the present invention is practically carried out.

As will become apparent as the description proceeds, the explanation will be made with respect to a process for producing an automotive side roof rail S (see FIG. 37) as an example of the final component or a shaped hollow product.

As is seen from FIGS. 1 to 4, the hydroforming device 1 comprises generally a female die 2 which has a cavity 2a formed therein, two sealing tools 3 which seal both open ends of a tubular work W, two supporting members 4 which stably support both end portions of the tubular work W while having a major portion of the tubular work W put in the cavity 2a of the female die 2, two feeding tubes 5 which feed and draw a hydraulic fluid into and from an interior Wa of the tubular work W whose ends are sealed by the sealing tools 3 and a male die 6 which presses the tubular work W in the cavity 2a of the female die 2. During pressing of the tubular work W by the male die 6, the interior Wa of the work W is kept filled with the hydraulic fluid of pressure P. For pressing the male die 6 against the work W, a ram R extending from a hydraulic actuator is connected to the male die 6.

As is seen from FIG. 4, the cavity 2a of the female die 2 is defined by two mutually facing vertical walls 2b, a bottom wall 2c and two slanted walls 2d each extending between the bottom wall 2c and the vertical wall 2b. The male die 6 is arranged to move upward and downward in the cavity 2a of the female die 2. The male die 6 comprises a work pressing main surface 6a and two projected side surfaces 6b which are located at lateral ends of the main surface 6a. As shown, each projected side surface 6b is generally perpendicular to the vertical wall 2b of the female die 2.

For producing the automotive side roof rail S from the tubular work W by using the above-mentioned hydroforming device 1, the following steps were carried out.

First, the tubular work W was set in the cavity 2a of the female die 2 and held stably by the supporting members 4. The tubular work W had a wall thickness of about 2.2 mm. More specifically, the work W was made of a steel of 370 MPa type, that is, a carbon steel tube of STKM11A specified by JIS (Japanese Industrial Standard) G 3445. Then, the sealing tools 3 were put into the open ends of the tubular work W to seal the same. Then, a hydraulic fluid was led into the interior Wa of the work W through the feeding tubes 5 and the interior of the work W was kept at a given pressure P that was 50 MPa. The pressure P was kept lower than a value that would induce expansion of the work W.

Then, as is seen from FIGS. 1 and 2 with the interior pressure P kept at 50 MPa, the male die 6 was lowered into the cavity 2a of the female die 2 to press the tubular work W at the work pressing main surface 6a. With these steps, the automotive side roof rail S was produced, which had a depressed hexagonal cross section as is understood from FIG. 5.

As is seen from FIG. 5, the depressed hexagonal cross section of the side roof rail S thus produced had a circumferential length that was smaller than that of the tubular work W. While, the thickness of the produced side roof rail S

became greater than that of a corresponding portion of the tubular work W except a bottom wall Sc of the rail S and its neighboring portion. That is, as is seen from FIG. 5, by applying the hydroforming process of the invention to the work W, the thickness of each vertical wall Sb of the rail S increased by about 9%, the thickness of each corner portion Se defined between the vertical wall Sb and a horizontal upper wall Sa increased by over 25% and even each rounded portion Sf defined between the vertical wall Sb and the slanted wall Sd showed a little increase in thickness.

In addition to the above, by using the above-mentioned hydroforming device 1, substantially identical hydroforming process was applied to a tubular work which was made of a steel of 590 MPa type and had a wall thickness of about 2.0 mm. Also, in this case, each rounded portion Sf defined between the vertical wall Sb and the slanted wall Sd showed a certain increase in thickness. This fact has revealed that even a tube of less malleable steel can be used as the work for the hydroforming process of the present invention.

For examining a mechanical strength of the side roof rail S thus produced, a test was carried out. That is, as is seen from FIG. 6, an elongate test piece S' was cut from the rail S, and two I-type steel blocks 7 were welded to respective ends of the test piece S' to provide an elongate test piece unit. The elongate test piece unit was put on two holders 8 which were spaced by 500 mm. Then, a center of the test piece unit was pressed down by a rounded pusher 9 of R50. That is, a load applied to the center of the test piece unit was gradually increased by the rounded head of the pusher 9.

FIG. 7 is a graph showing the results of the test in terms of a relation between the load applied by the rounded pusher 9 and a stroke of the pusher 9. For comparison, similar test was applied to a reference test piece which showed no increase in thickness. As is seen from this graph, the test piece S' produced in accordance with the present invention exhibited the maximum flexural rigidity (viz., about 4200 Kgf) that is greater than that (viz., about 2600 Kgf) of the reference test piece by about 64%. Other tests revealed that as is seen from the graph of FIG. 8, when the thickness of the vertical walls Sb increased by over 3%, the mechanical strength showed a satisfied value.

Referring to FIG. 9, there is schematically shown a female die 22 employed in a hydroforming device 21 with which a method of a second embodiment of the present invention is carried out.

As is seen from the drawing, the female die 22 is formed with an axially extending stepped portion 22g between each vertical wall 22b and the adjacent slanted wall 22d. Preferably, the size of the stepped portion 22g is smaller than the thickness of the tubular work W and greater than one tenth (viz.,  $\frac{1}{10}$ ) of the thickness of the work W. Denoted by numeral 22a is a cavity defined by the female die 22. Several tests have revealed that the presence of such stepped portions 22g lessens the possibility of producing undesired buckling of the tubular work W during the forming process. Furthermore, the tests have revealed that the presence of the stepped portions 22g assuredly reduces the stroke length of the male die.

Referring to FIGS. 10 and 11, particularly FIG. 10, there is shown but partially and in a sectional manner a female die 32 employed in a hydroforming device 31 with which a method of a third embodiment of the present invention is carried out.

As is seen from FIG. 10, in this female die 32, there is formed, between each vertical wall 32b and the corresponding slanted wall 32d, with an extra slanted wall 32g that

defines an angle "θ" relative to the vertical wall 32b. Preferably, the angle "θ" is within a range from 0 to 45°. Denoted by numeral 32a is a cavity defined by the female die 32. Tests have revealed that due to presence of such extra slanted walls 32g, the friction inevitably produced between the wall of the female die 32 and the male die 6 is reduced and the pressing load applied by the male die 6 is evenly transmitted to the entire construction of the work W.

For finding a desired value of the angle "θ" in case wherein the hydroforming process reduces the circumferential length of the tubular work W by 3%, a test was carried out. In this test, many tubular works were subjected to the hydroforming process by using many female dies 32 that had different values of the angle "θ", and the rate of increase in thickness of the vertical wall Sb of each product (viz., side rail roof S) was measured.

The result of this test is depicted in FIG. 11. As is seen from this graph, when the angle "θ" exceeded about 50°, the rate of increase in thickness of the vertical wall Sb of the product S became lower than 3%.

Referring to FIGS. 12 and 13, there is schematically shown a hydroforming device 41 with which a method of a fourth embodiment of the present invention is carried out. This forming device 41 is designed to make a hydroformed product SA having a rectangular cross section, as shown in FIG. 14.

In this fourth embodiment, two male dies 46 are employed, which are arranged to move toward and away from each other in a cavity 42a formed in a female die 42. Two sealing tools 3, two supporting members 4 and two feeding tubes 5 are arranged in substantially the same manner as in the case of the above-mentioned first embodiment 1 of FIGS. 1 and 2.

For producing the product SA, a tubular work W was prepared. The tubular work W was the same as the work W used in the above-mentioned first embodiment. The tubular work W was set in the cavity 42a and held stably by the supporting members 4. Then, the sealing tools 3 were put into the open ends of the tubular work W to seal the same. Then, a hydraulic fluid was led into the interior Wa of the work W through the feeding tubes 5 and the interior of the work W was kept at a given pressure that was 50 MPa.

Then, as is seen from FIG. 13, with the interior pressure kept constant, the two male dies 46 were moved toward each other to press the tubular work W from both sides. With these steps, the product SA as shown in FIG. 14 was provided, which had a rectangular cross section.

As is seen from FIG. 14, the product SA had a circumferential length that was smaller than that of the tubular work W. While, the thickness of each vertical wall SAb became greater than that of a corresponding portion of the tubular work W. In fact, the thickness of each vertical wall SAb was much greater than that of the vertical wall Sb of the product S produced in the above-mentioned first embodiment. That is, the thickness of each vertical wall SAb increased by about 20%. Furthermore, no reduction in thickness at the four corners SAE was found. That is, the thickness of each corner SAE increased by about 30%.

In addition to the above, substantially identical hydroforming process was applied to a tubular work which was made of a steel of 590 MPa type and had a wall thickness of about 2.0 mm. Also in this case, sufficient increase in thickness of the product was found. This fact has revealed that even a tube of less malleable steel can be used as the work for the hydroforming process of the present invention.

Referring to FIG. 15, there is schematically shown a hydroforming device 51 with which a method of a fifth embodiment of the present invention is carried out.

Similar to the device 1 for the above-mentioned first embodiment, the hydroforming device 51 for this fifth embodiment comprises generally a female die 53 and a male die 52. The female die 53 has a generally U-shaped cross section and has a cavity 53a formed therein. The male die 52 is connected to a ram R (see FIG. 3) of a hydraulic actuator, so that the male die 52 can move up and down in the cavity 53a of the female die 53.

As shown in the drawing, the male die 52 is formed at lateral ends of its major work surface 52a with respective projections 52b that project into the cavity 53a. Each projection 52b has a triangular cross section and has a sloped work surface 52c that faces the cavity 53a. Furthermore, each projection 52b has a leading edge that is rounded. Preferably, the radius of curvature of the rounded edge is about a half of the thickness of a tubular work W. In the illustrated embodiment, the radius of curvature is about 1 mm.

For finding a desired shape of the male die 52 to produce a satisfied hollow product M1 from the tubular work W, four male dies 52 were prepared. These male dies 52 were different in shape of the projections 52b. That is, the length "L" of the sloped work surface 52c and the angle "α" defined by the sloped work surface 52c relative to a vertical wall 53b of the female die 53 were different in the four male dies 52.

By taking the following steps, four products M1 were provided from respective tubular works W through the hydroforming process using the four male dies 52.

First, each tubular work W was set in the cavity 53a of the female die 53 and stably held. Each tubular work W was made of a steel of 370 MPa type and was 101.6 mm in diameter and 2.0 mm in thickness. Then, the interior of the tubular work W was filled a hydraulic fluid and kept at 20 MPa. Then, the male die 52 was lowered into the cavity 53a to press the tubular work W. With these steps, the four products M1 were provided, each product M1 having a depressed octagonal cross section as is seen from the drawing. In these four products M1, the thickness of two sloped upper portions M1a was measured for investigating a thickness change of the portions M1a due to the hydroforming process. These two sloped upper portions M1a were mainly shaped by the projections 52b of the male die 52.

The result of the investigating is shown in TABLE-1. As is seen from the table, when using the first male die 52 (viz.,  $α=141^\circ$ ,  $D=5.0$ ), the thickness of each sloped upper portion M1a increased by 30%, and when using the second male die 52 (viz.,  $α=153^\circ$ ,  $D=5.6$ ), the thickness of the portion M1a increased by 15% and when using the third male die 52 (viz.,  $α=153^\circ$ ,  $D=6.7$ ), the thickness of the portion M1a increased by 10%. In case of the first, second and third male dies 52, it was further found that with increase of the pressing stroke of the male die 52, the circumferential length of the product M1 decreased and the thickness of each sloped upper portion M1a increased. While, when using the fourth male die 52 (viz.,  $α=124^\circ$ ,  $D=9.0$ ), the sloped upper portions M1a of the product M1 showed creases. That is, in case of this fourth male die 52, with increase of the pressing stroke of the male die 52, creases gradually appeared at the two sloped upper portions M1a of the product M1.

FIG. 16 is a graph showing the result in case of using the second male die 52 (viz.,  $α=153^\circ$ ,  $D=5.6$ ). That is, the graph plots the thickness increasing rate of the sloped upper portions M1a relative the pressing stroke of the second male die 52. As is seen from this graph, with increase of the pressing stroke of the second male die 52, the thickness of

the two sloped upper portions M1a increased and at the same time, the thickness of two vertical wall portions M1b (see FIG. 15) of the product M1 increased. The two vertical wall portions M1b were mainly shaped by the vertical walls 53b of the female die 53. As is seen, once the pressing stroke of the male die 52 exceeded 20 mm, the thickness increasing rate of the sloped upper portions M1a sharply increased as compared with that of the vertical wall portions M1b. That is, the thickness of the wall portions M1a that were mainly shaped by the projections 52b of the male die 52 increased exclusively.

Referring to FIG. 17, there is schematically shown a hydroforming device 61 with which a method of a sixth embodiment of the present invention is carried out.

As shown, the device 61 of this embodiment comprises generally a female die 64 and two male dies 62 and 63 which are arranged to move toward and away from each other in a cavity 64a of the female die 64. Although not shown in the drawing, the two male dies 62 and 63 are powered by a hydraulic actuator.

The male die 62 is formed at lateral ends of its major work surface 62a with respective projections 62b that project into the cavity 64a. Each projection 62b has a triangular cross section and has a sloped work surface 62c that faces the cavity 64a. The length "L1" of the sloped work surface 62c is 11.2 mm and the angle "α1" defined by the sloped work surface 62c relative to a vertical wall 64b of the female die 64 is 153°.

The other male die 63 is formed at lateral ends of its major work surface 63a with respective projections 63b that project into the cavity 64a. Each projection 63b has a triangular cross section and has a sloped work surface 63c. The length "L2" of the sloped work surface 63c is 11.2 mm and the angle "α2" defined by the sloped work surface 63c relative to the vertical wall 64b of the female die 64 is 117°.

By using the hydroforming device 61, a tubular work W was subjected to a hydroforming process. The work W was the same as that used in the above-mentioned fifth embodiment. The tubular work W was set in the cavity 64a of the female die 64 and stably held. Then, the interior of the work W was filled with a hydraulic fluid and kept at a certain pressure that did induce a free bulging of the work W. The certain pressure was lower than a critical level that is calculated from the following equation:

$$CL=t_0 \times Sy \times 1.6 \quad (1)$$

Wherein:

CL: critical level (MPa)

$t_0$ : thickness of tubular work (mm)

Sy: yield strength (MPa)

Then, the two male dies 62 and 63 are moved toward each other to press the tubular work W.

With these steps, a hollow product M2 was provided that had a depressed octagonal cross section as is seen from the drawing.

The thickness of two sloped upper portions M2a and that of two sloped lower portions M2b of the product M2 were measured for investigating the thickness change of those portions M2a and M2b due to the hydroforming process.

The result of the investigating is shown in TABLE-2. As is seen from this table, due to the hydroforming process using the hydroforming device 61 of the sixth embodiment, the thickness of the upper sloped portions M2a and that of the lower sloped portions M2b increased by 10% and 20% respectively. More specifically, the thickness of the portions

**M2a** and **M2b** that were mainly shaped by the projections **62b** and **63b** of the upper and lower male dies **62** increased exclusively. In addition to this, it was further found that due to the hydroforming process by the device **61**, the thickness of vertical walls **M2c** of the product **M2** increased also.

Because the increase in thickness of the specified portions induces a work-hardening of the same, the mechanical strength of the product **M2** is remarkably increased due to combination of the thickness increase and work-hardening.

If the product **M2** thus provided is put into the hydroforming device **61** and set in the cavity **64a** with the two walls **M2c** thereof facing the upper and lower male dies **62** and **63**, pressing of the product **M2** by the two male dies **62** and **63** can provide the product **M2** with a generally square cross section. Furthermore, with this process, the neighboring walls of the product **M2** can have different thickness.

Referring to FIG. 18, there is schematically shown a hydroforming device **71** with which a method of a seventh embodiment of the present invention is carried out.

The device **71** of this seventh embodiment is substantially the same as the device **51** of the above-mentioned fifth embodiment of FIG. 15 except that in the seventh embodiment the male die **72** is formed with only one projection **72b**. That is, the projection **72b** is provided at one lateral end of the major work surface **72a** of the male die **72**. The projection **72b** has a triangular cross section and has a sloped work surface **72c**. The male die **72** moves in a cavity **73a** of the female die **73**. The length "L" of the sloped work surface **72c** is 11.2 mm and the angle "α" defined by the sloped work surface **72c** relative to a vertical wall **73b** of the female die **73** is 153°.

By using the hydroforming device **71**, a tubular work **W** was subjected to a hydroforming process. The work **W** was the same as that used in the above-mentioned fifth embodiment. The work **W** was set in the cavity **73a** of the female die **73** and stably held. Then, the interior of the work **W** was filled with a hydraulic fluid and kept at a pressure that did make a substantial promotion of a free bulging of the work **W**. Then, the male die **72** was lowered to press the work **W**. With these steps, a product **M3** was provided that had a depressed heptagonal cross section as is seen from the drawing.

The thickness of a sloped upper portion **M3a** of the product **M3** was measured for investigating the thickness change of that portion **M3a** due to the hydroforming process.

The result of the investigating is shown in TABLE-3. As is seen from this table, due to the hydroforming process using the hydroforming device **71** of the seventh embodiment, the thickness of the sloped upper portion **M3a** increased by 10%. In addition, it was found that due to the hydroforming process by the device **71**, the thickness of vertical walls **M3b** of the product **M3** increased also.

Referring to FIG. 19, there is schematically shown a hydroforming device **81** with which a method of an eighth embodiment of the present invention is carried out.

The device **81** of this eighth embodiment is substantially the same as the device **61** of the above-mentioned sixth embodiment of FIG. 17 except that in the eighth embodiment each of the upper and lower male dies **82** and **83** is formed with only one projection **82b** or **83b**. As shown, the projections **82b** and **83b** are positioned at opposite sides with respect to a center axis of the device **81** and each projection **82b** or **83b** is provided at one lateral end of the major work surface **82a** or **83a** of the male die **82** or **83**. The projection **82b** or **83b** has a triangular cross section and has a sloped work surface **82c** or **83c**. The upper and lower male dies **82** and **83** move toward and away from each other in a cavity

**84a** of the female die **84**. The length "L1" of the sloped work surface **82c** of the upper male die **82** is 11.2 mm and the angle "α1" defined by the sloped work surface **82c** relative to a vertical wall **84b** of the female die **84** is 153°. While, the length "L2" of the sloped work surface **83c** of the lower male die **83** is 11.2 mm and the angle "α2" defined by the sloped work surface **83c** relative to a vertical wall **84b** of the female die **84** is 117°.

By using the hydroforming device **81**, a tubular work **W** was subjected to a hydroforming process. That is, the work **W** was set in the cavity **84a** of the female die **84** and held stably. Then, the interior of the work **W** was filled with a hydraulic fluid and kept at a certain pressure that did not make a substantial promotion to a free bulging of the work **W**. Then, the two male dies **82** and **83** are moved toward each other to press the tubular work **W**. With these steps, a product **M4** was provided that had a depressed hexagonal cross section as is seen from the drawing.

The thickness of a sloped upper portion **M4a** and that of a sloped lower portion **M4b** of the product **M4** were measured for investigating the thickness change of these portions **M4a** and **M4b** due to the hydroforming process.

The result of this investigation is shown in TABLE-4. As is seen from this table, due to the hydroforming process using the hydroforming device **81**, the thickness of the upper and lower sloped portions **M4a** and **M4b** increased by 10% and 20% respectively. More specifically, the thickness of the portions **M4a** and **M4b** that were mainly shaped by the projections **82b** and **83b** of the male dies **82** and **83** increased exclusively. In addition to this, it was further found that due to the hydroforming process by the device **81**, the thickness of vertical walls **M4c** of the product **M4** increased also.

Referring to FIG. 20, there is schematically shown a hydroforming device **91** with which a method of a ninth embodiment of the present invention is carried out.

The device **91** used in this ninth embodiment is substantially the same as the device **61** of the above-mentioned sixth embodiment of FIG. 17 except that in the ninth embodiment the projections **93b** of the lower male die **93** are different from those **63b** of the lower male die **63** of the sixth embodiment. That is, in the ninth embodiment, the length "L2" of each sloped work surface **93c** is 11.2 mm, but the angle "α2" defined by the sloped work surface **93c** relative to the vertical wall **94b** of the female die **94** is 153° which is the same as the sloped work surface **92c** of each projection **92b** of the upper male die **92**.

By using the hydroforming device **91**, a tubular work **W** was subjected to a hydroforming process. The work **W** used in this embodiment was substantially the same as that used in the fifth embodiment except that in this ninth embodiment the work **W** was made of a steel of 590 MPa type. The tubular work **W** was set in the cavity **94a** of the female die **94** and stably held. Then, the interior of the work **W** was filled with a hydraulic fluid and kept at about 20 MPa. Then, the two male dies **92** and **93** are moved toward each other to press the tubular work **W**. During this pressing, the hydraulic pressure in the work **W** increased. However, by using a leak-off valve (not shown), rapid increase of the pressure was suppressed. For this pressing, the maximum pressing stroke of each male die **92** or **93** was so determined as to cause a product **M5** (see FIG. 21) to have a circumferential length smaller than that of the non-pressed tubular work **W**. At the maximum pressing stroke of each male die **92** or **93**, the pressure of the fluid in the work **W** showed a level above 30 MPa.

With these steps, the product **M5** was provided that had a depressed octagonal cross section as is seen FIG. 21.

The thickness of two sloped upper portions **M5a**, the thickness of two sloped lower portions **M5b** and the thickness of two vertical portions **M5c** of the product **M5** were measured, which were 2.30 mm, 2.30 mm and 2.20 mm respectively. That is, the sloped upper portions **M5a** increased by 15%, the sloped lower portions **M5b** increased 15% and the vertical portions **M5c** increased by 10% in thickness. It was further found that portions (viz., upper and lower horizontal wall portions) other than the above-mentioned portions **M5a**, **M5b** and **M5c** showed no change in thickness.

Referring to FIG. 22, there is schematically shown a hydroforming device **101** with which a method of a tenth embodiment of the present invention is carried out.

The device **101** used in this tenth embodiment is substantially the same as the device **81** of the above-mentioned eighth embodiment of FIG. 19 except that in the tenth embodiment the projection **103b** of the lower male die **103** is different from that **83b** of the lower male die **83** of the eighth embodiment. That is, in the tenth embodiment, the length "L2" of the sloped work surface **103c** is 11.2 mm, but the angle "α2" defined by the sloped work surface **103c** relative to the vertical wall **104b** of the female die **104** is 153° which is the same as the sloped work surface **102c** of the projection **102b** of the upper male die **102**.

By using the hydroforming device **101**, a tubular work **W** was subjected to a hydroforming process. The work **W** used in this embodiment was the same as that used in the above-mentioned ninth embodiment. The tubular work **W** was set in the cavity **104a** of the female die **104** and stably held. The interior of the work **W** was filled with a hydraulic fluid and kept at about 20 MPa. Then, the two male dies **102** and **103** are moved toward each other to press the tubular work **W**. For this pressing, the maximum pressing stroke of each male die **102** or **103** was so determined as to cause a product **M6** (see FIG. 23) to have a circumferential length smaller than that of the non-pressed tubular work **W**. At the maximum pressing stroke of each male die **102** or **103**, the pressure of the fluid in the work **W** showed a value above 30 MPa.

With these steps, the product **M6** was provided that had a depressed hexagonal cross section, as is seen from FIG. 23.

The thickness of a sloped upper portion **M6a**, that of a sloped lower portion **M6b** and that of two vertical portions **M6c** and **M6d** of the product **M6** were measured, which were 2.24 mm, 2.24 mm, 2.16 mm and 2.20 mm respectively. That is, the sloped upper portion **M6a** increased by 12%, the sloped lower portion **M6b** increased by 12%, the vertical portion **M6c** increased by 8% and the other vertical portion **M6d** increased by 10% in thickness. It was further found that portions (viz., upper and lower horizontal wall portions) other than the above-mentioned portions **M6a**, **M6b**, **M6c** and **M6d** showed no change in thickness.

Referring to FIG. 24, there is shown a reference hydroforming device **111**, which was provided for proving the improvement achieved by the present invention.

The device **111** is substantially the same as the device **51** used in the above-mentioned fifth embodiment of FIG. 15 except that in this reference device **111a** cavity **113a** of the female die **113** has an entirely flat bottom **113c**, as shown. The length "L" of the sloped work surface **112c** of each projection **112b** is 11.2 mm and the angle "α" defined by the sloped work surface **112c** relative to the vertical wall **113b** of the female die **113** is 153°.

By using the reference device **111**, a tubular work was subjected to a hydroforming process. The work **W** was the same as the work **W** used in the above-mentioned ninth and

tenth embodiments. Steps of the hydroforming process were substantially the same as those of the ninth and tenth embodiments.

With these steps, a product **M7** was provided, that had a depressed hexagonal cross section, as is seen from FIG. 25.

The thickness of a right side sloped upper portion **M7a** and that of a left side vertical wall **M7c** of the product **M7** were measured, which were 2.30 mm and 2.20 mm respectively. That is, these portions **M7a** and **M7c** increased by 15% and 10% in thickness respectively. However, it was found that portions other than those portions **M7a** and **M7b** showed no change in thickness. That is, in case of this reference device **111**, the product **M7** failed to have continuous vertical and sloped portions that were both increased in thickness.

For the above, it has been revealed that if the sloped surface **92c**, **93c**, **102c** or **103c** of each projection **92b**, **93b**, **102b** or **103b** of the male die **92**, **93**, **102** or **103** is constructed to satisfy the following equations, a desired result is expected for producing the shaped hollow product **M5** or **M6**.

$$4 \leq L/t_0 \leq 7.5 \quad (2)$$

$$\alpha \geq 10 \times (L/t_0) + 68 \quad (3)$$

wherein:

**L**: length of the sloped surface

**t<sub>0</sub>**: initial thickness of the tubular work

α: angle between the sloped surface and the vertical wall.

Referring to FIG. 26, there is schematically shown a hydroforming device **121** with which a method of an eleventh embodiment of the present invention is carried out. As will be described in detail hereinafter, the device **121** of this embodiment is constructed to shape a tubular work **W** into a hollow square product **M8** (see FIG. 27) with four rounded corners **M8a**.

As is seen from FIG. 26, the device **121** used in this eleventh embodiment comprises generally fixed lower and upper dies **122** and **123** which are mounted on each other to define therebetween a longitudinally extending cavity **121a**. Each fixed die **122** or **123** is formed at laterally spaced internal portions with longitudinally extending concave surfaces **122a** or **123a**. These concave surfaces **122a** and **123a** are used for shaping the four rounded corners **M8a** of the product **M8**.

The two fixed dies **122** and **123** are respectively formed with vertical slots **122b** and **123b** in which lower and upper male dies **124** and **125** are movably received. The two fixed dies **122** and **123** are vertically spaced from each other to define therebetween horizontal slots **126a** and **126b** in which left and right male dies **127** and **128** are movably received. These four male dies **124**, **125**, **127** and **128** are used for shaping the four flat wall portions **M8b** of the product **M8**.

As is seen from FIG. 26, each slot **122b**, **123b**, **126a** or **126b** is exposed to the cavity **121a** at longitudinally extending ridges **P1** that constitute circumferentially terminal ends of the corresponding concave surfaces **122a** and **123a**. That is, each ridge **P1** constitutes an inside edge of the corresponding slot **122b**, **123b**, **126a** or **126b**.

It is now to be noted that in this eleventh embodiment **121**, the ridges **P1** are shaped and sized to satisfy the following geometrical conditions.

That is, an imaginary straight line "T1" that passes through neighboring two ridges **P1** and **P1** of each slot extends outside of the cavity **121a** defined by the lower and upper female dies **122** and **123**. In other words, the imaginary straight line "T1" does not pass any area of the cavity

121a. When the male dies 124, 125, 127 and 128 are brought to their frontmost work positions, the flat work surface (no numeral) of each male die 124, 125, 127 or 128 becomes coincident with the corresponding imaginary straight line "T1". In this condition, the work surface of each male die 124, 125, 127 or 128 is smoothly mated with the ridges P1, that is, the circumferentially terminal ends of the concave surfaces 122a and 123a.

By using the hydroforming device 121, a tubular work W was subjected to a hydroforming process. The work W was made of a steel of 370 MPa type and was 123 mm in diameter and 2 mm in thickness. That is, the work W was set in the cavity 121a of the fixed dies 122 and 123, and the male dies 124, 125, 127 and 128 were moved to their rest position and then, the work W was stably held in the cavity 121a. Then, the interior of the work W was filled with a hydraulic fluid and the pressure in the work W was increased to and kept at 10.1 MPa. Then, the male dies 124, 125, 127 and 128 were moved to their work or press positions to press the work W. During this pressing, the pressure in the work W gradually increased, and at the maximum pressing stroke of each male die, the pressure in the work W was increased to a level of 24.8 MPa.

With these steps, a hollow square product M8 was provided that had a square cross section with four rounded corners, as is seen from FIG. 27. The radius of curvature of each corner M8a was 8 mm, the height was 100 mm and the width was 100 mm.

The thickness of various portions "a to j" of one rounded corner M8a and its neighboring flat wall portion M8b of the product M8 was measured, as is seen from FIG. 28.

FIG. 29 is a graph showing the result of the thickness measuring, that plots the thickness of such portions "a to j". For comparison, the result provided by a conventional hydroforming device having no moving dies is also plotted. As is seen from this graph, in the conventional one, the thickness of the rounded corner M8a reduced by 20% at most, while in case of the product M8 of the invention, the thickness of such corner M8a increased by 20% at most. That is, by using the hydroforming device 121 of the eleventh embodiment, undesired thickness reduction in the corner was suppressed.

Referring to FIG. 30, there is schematically shown a hydroforming device 131 with which is a method of a twelfth embodiment of the present invention is carried out. As will be described in detail hereinafter, the device 131 of this embodiment is constructed to shape a tubular work W into a hollow square product M9 (see FIG. 32) with four projected round corners M9a.

As is seen from FIG. 30, the device 131 used in this twelfth embodiment comprises generally fixed lower and upper dies 133 and 134 which are mounted on each other to define therebetween a longitudinally extending cavity 131a.

Each fixed die 133 or 134 is formed at laterally spaced internal portions with longitudinally extending concave surfaces 133a or 134a.

The two fixed dies 133 and 134 are respectively formed with vertical slots 133b and 134b in which lower and upper male dies 135 and 136 are movably received. The two fixed dies 133 and 134 are vertically spaced from each other to define therebetween horizontal slots 137a and 137b in which left and right male dies 138 and 139 are movably received.

As shown, each male die 135, 136, 138 or 139 is formed at lateral ends of the work surface 135a, 136a, 138a or 139a with respective concave recesses 135b, 136b, 138b or 139b.

As is understood from FIG. 31, one concave surface 134a or 133a of the fixed female die 134 or 133 and neighboring two

concave recesses 136b and 138b, 136b and 139b, 138b and 135b or 135b and 139b of the corresponding male dies 136, 138, 139 and 135 are used for shaping one projected round corner M9a of the product M9.

As is seen from FIG. 30, each slot 133b, 134b, 137a or 137b is exposed to the cavity 131a at longitudinally extending ridges P2 that constitute circumferentially terminal ends of the corresponding concave surfaces 133a and 134a. That is, each ridge P2 constitutes an inside edge of the corresponding slot 133b, 134b, 137a or 137b.

It is now to be noted that in this twelfth embodiment 131, the ridges P2 are so shaped and sized as to satisfy the following geometrical conditions.

That is, as is seen from FIG. 30, an imaginary straight line "T2" that passes through neighboring two ridges P2 and P2 of each slot extends outside of the cavity 131a defined by the lower and upper fixed female dies 133 and 134. In other words, the imaginary straight line "T2" does not pass any area of the cavity 131a. As is seen from FIG. 31, when the male dies 136, 138, 135 and 139 are brought to their frontmost work positions, the outside edge of each concave recess 136b, 138b, 135b or 139b becomes coincident with the corresponding imaginary straight line "T2". In this condition, the outside edge of each concave recess 136b, 138b, 135b or 139b is smoothly mated with the ridges P2, that is, the circumferentially terminal ends of the concave surfaces 134a and 133a.

By using the hydroforming device 131, a tubular work W was subjected to a hydroforming process. The work W was made of a steel of 370 MPa type and was 140 mm in diameter and 2 mm in thickness. That is, the work W was set in the cavity 131a of the fixed dies 133 and 134, and the male dies 135, 136, 138 and 139 were moved to their rest positions and then, the work W was stably held in the cavity 131a. Then, the interior of the work W was filled with a hydraulic fluid and the pressure in the work W was increased to and kept at 10.1 MPa. Then, the male dies 135, 136, 138 and 139 were moved toward their work or press positions to press the work W while keeping the internal pressure of the work W at 20.2 MPa. At the maximum pressing stroke of each male die, the pressure in the work W was increased to a level of 24.8 MPa.

With these steps, a hollow square product M9 was provided, that had a generally square cross section with four projected round corners, as is seen from FIG. 32. The radius of curvature of each corner M9a was 10 mm, the height was 100 mm and the width was 100 mm.

The thickness of various portions "a to j" of one projected round corner M9a and its neighboring flat wall portion M9b of the product M9 was measured, as is seen from FIG. 33.

FIG. 36 is a graph showing the result of the thickness measuring, that plots the thickness of such portions "a to j".

For proving the improvement achieved by the method of the twelfth embodiment, a reference method was carried out by using a hydroforming device 141 shown in FIG. 34.

As is shown in the drawing, the device 141 comprises fixed lower and upper dies 143 and 144, lower and upper male dies 145 and 146 and left and right male dies 148 and 149 which are arranged in substantially the same manner as those of the above-mentioned device 131 of the twelfth embodiment of FIG. 30.

Each fixed die 143 or 144 is formed at laterally spaced internal portions with longitudinally extending concave surfaces 143a or 144a.

Each male die 145, 146, 148 or 149 is formed with a flat work surface 145a, 146a, 148a or 149a.

As is seen from FIGS. 34 and 35, each slot 143b, 144b, 147a or 147b is exposed to the cavity 141a at longitudinally

extending ridges P3 that constitute circumferentially terminal ends of the corresponding concave surfaces 143a and 144a. That is, each ridge P3 constitutes an inside edge of the corresponding slot 143b, 144b, 147a or 147b.

In this reference device 141, the ridges P3 are so shaped and sized as to satisfy the following geometrical conditions.

That is, as is seen from FIG. 34, an imaginary straight line "T3" that passes through neighboring two ridges P3 and P3 of each slot extends inside (not outside) of the cavity 141a defined by the lower and upper fixed female dies 144 and 144. In other words, the imaginary straight line "T3" passes through the projected part of the cavity 121a, which is defined by the concave surface 144a or 143a of the female die 144 or 143. When the male dies 145, 146, 148 and 149 are brought to their frontmost work positions, the flat work surface 145a, 146a, 148a or 149a of each male die becomes coincident with the corresponding imaginary straight line "T3". In this condition, the work surface 145a, 146a, 148a or 149a of each male die is mated with the ridges P3, as is seen from FIG. 35.

By using the reference device 141, a tubular work W was subjected to a hydroforming process. The work W and the hydroforming steps were the same as those used in the above-mentioned twelfth embodiment. With this, a hollow square product MR was provided, that was similar in construction to the product M9 provided according to the twelfth embodiment. The thickness of various portions "a to j" of the product MR was measured. The result of the thickness measurement is plotted in the graph of FIG. 36.

As is seen from this graph, in the product M9 according to the twelfth embodiment, the thickness of the projected round corner M9a increased by about 15%, while in the product MR according to the reference device 141, thickness increase was now found and a crack was produced at the portion "g".

The entire contents of Japanese Patent Applications 11-083658 (filed Mar. 26, 1999), 11-183920 (filed Jun. 29, 1999), 11-366894 (filed Dec. 24, 1999) and 2000-49476 (filed Feb. 25, 2000), are incorporated herein by reference.

Although the invention has been described above with reference to the embodiments, the invention is not limited to such embodiments as described hereinabove. Various modifications and variations of such embodiments may be carried out by those skilled in the art, in light of the above description.

TABLE 1

| Hydraulic forming device | Angle of projection $\alpha(^{\circ})$ | Length of sloped work surface L (mm) |     | Initial thickness $t_0$ (mm) | Ratio (D) $(L/t_0)$ | Increasing rate of thickness $10D + 68$ (%) |     |                    |
|--------------------------|----------------------------------------|--------------------------------------|-----|------------------------------|---------------------|---------------------------------------------|-----|--------------------|
|                          |                                        | FIG. 15                              | 141 | 10.0                         | 2.0                 | 5.0                                         | 118 | 3                  |
|                          |                                        | 153                                  |     | 11.2                         | 2.0                 | 5.6                                         | 124 | 15                 |
|                          |                                        | 153                                  |     | 13.4                         | 2.0                 | 6.7                                         | 135 | 10                 |
|                          |                                        | 124                                  |     | 18.0                         | 2.0                 | 9.0                                         | 158 | (Creases appeared) |

TABLE 2

| Hydraulic forming device | Angle of projection $\alpha(^{\circ})$ | Length of sloped work surface L (mm) | Initial thickness $t_0$ (mm) | Ratio (D) $(L/t_0)$ | Increasing rate of thickness $10D + 68$ (%) |     |    |
|--------------------------|----------------------------------------|--------------------------------------|------------------------------|---------------------|---------------------------------------------|-----|----|
| FIG. 17                  | 62b                                    | $\alpha:1:153$                       | L1:11.2                      | 2.0                 | 5.6                                         | 124 | 10 |
| 10                       | 63b                                    | $\alpha:2:117$                       | L2:11.2                      | 2.0                 | 5.6                                         | 124 | 2  |

TABLE 3

| Hydraulic forming device | Angle of projection $\alpha(^{\circ})$ | Length of sloped work surface L (mm) | Initial thickness $t_0$ (mm) | Ratio (D) $(L/t_0)$ | Increasing rate of thickness $10D + 68$ (%) |    |
|--------------------------|----------------------------------------|--------------------------------------|------------------------------|---------------------|---------------------------------------------|----|
| FIG. 18                  | 153                                    | 11.2                                 | 2.0                          | 5.6                 | 124                                         | 10 |

TABLE 4

| Hydraulic forming device | Angle of projection $\alpha(^{\circ})$ | Length of sloped work surface L (mm) | Initial thickness $t_0$ (mm) | Ratio (D) $(L/t_0)$ | Increasing rate of thickness $10D + 68$ (%) |     |    |
|--------------------------|----------------------------------------|--------------------------------------|------------------------------|---------------------|---------------------------------------------|-----|----|
| FIG. 19                  | 82b                                    | $\alpha:1:153$                       | L1:11.2                      | 2.0                 | 5.6                                         | 124 | 10 |
| 30                       | 83b                                    | $\alpha:2:117$                       | L2:11.2                      | 2.0                 | 5.6                                         | 124 | 2  |

What is claimed is:

1. Method of forming a tubular work into a shaped hollow product by using hydroforming process, comprising: preparing female and male dies, said female die having a longitudinally extending cavity which has a polygonal cross section when receiving said male die; placing said tubular work in said cavity of the female die; feeding the interior of said tubular work with a hydraulic fluid; increasing the pressure of the hydraulic fluid to a given level, said given level being less than a critical level that causes a bulging of said tubular work; pressing said male die against said tubular work to deform the same while keeping the hydraulic fluid at said given level, thereby forming a shaped hollow product that has a polygonal cross section that conforms to that of said cavity; and continuing the pressing by the male die until a circumferential length of said shaped hollow product becomes shorter than that of said tubular work.
2. Method as claimed in claim 1, in which said given level of said hydraulic fluid is kept at least until the time when the pressing of said male die against said tubular work provides said tubular work with a rounded corner portion.
3. Method as claimed in claim 1, further comprising, before feeding the hydraulic fluid into said tubular work, holding said tubular work stably in said cavity.
4. Method as claimed in claim 1, in which the pressing of said male die against the tubular work is continued until a given portion of said shaped hollow product becomes thicker than a corresponding portion of said tubular work.
5. Method as claimed in claim 1, in which the polygonal cross section of said cavity is tetragonal or greater polygonal cross section.

6. Method as claimed in claim 1, in which said male die has a work surface that directly contacts an outer surface of said tubular work upon pressing of said male die against said tubular work, said work surface including a major flat surface and at least one sloped surface that are angled relative to each other, so that upon pressing of said male die, said major flat surface and said sloped surface provide said shaped hollow product with neighboring two angled walls.

7. Method as claimed in claim 6, in which the pressing of said male die against said tubular work is continued until at least one of said neighboring two angled walls of the product becomes thicker than a corresponding portion of said tubular work.

8. Method as claimed in claim 7, in which the pressing of said male die against said tubular work is continued until the thickness of the selected wall of the product becomes thicker than the corresponding portion of said tubular work by over 3%.

9. Method as claimed in claim 1, in which said male die includes two male die members which are arranged to put therebetween said tubular work and movable toward and away from said tubular work, each male die member having a work surface that directly contacts an outer surface of said tubular work upon pressing against said tubular work, so that upon pressing, the work surfaces of said two male die members form opposed walls of said shaped hollow product.

10. Method as claimed in claim 9, in which each of the work surfaces of the two die male members includes a major flat surface and at least one sloped surface that are angled relative to each other, so that upon pressing of the two male die members against the tubular work, said major flat surface and said sloped surface provide each of said opposed walls of the shaped hollow product with neighboring two angled wall portions.

11. Method as claimed in claim 10, in which the critical level of said hydraulic fluid in said tubular work is calculated from the following equation:

$$CL=t0 \times Sy \times 0.6$$

Wherein:

CL: critical level (MPa)

t0: thickness of tubular work (mm)

Sy: yield strength (MPa).

12. Method as claimed in claim 11, in which the sloped surface of the work surface of each male die members defines an obtuse angle relative to the corresponding major flat surface.

13. Method as claimed in claim 12, in which the pressing of the male die members against the tubular work is continued until the neighboring two angled wall portions of each of the opposed walls of the product become thicker than corresponding portions of said tubular work.

14. Method as claimed in claim 13, in which the pressing of the male die members against the tubular work is continued until the neighboring two angled wall portions of each of the opposed walls of the product become thicker than the corresponding portions of said tubular work by over 3%.

15. Method as claimed in claim 1, in which said female die includes four longitudinally extending concave surfaces which face said cavity, in which said male die includes four male die members which are movably received in respective slots formed in said female die, in which each slot is exposed to the cavity at longitudinally extending ridges that constitute circumferentially terminal ends of the corresponding concave surfaces, and in which an imaginary straight line

that passes through neighboring two of said ridges extends outside of said cavity.

16. Method as claimed in claim 15, in which the critical level of said hydraulic fluid in said tubular work is calculated from the following equation:

$$CL=t0 \times Sy \times 0.6$$

Wherein:

CL: critical level (MPa)

t0: thickness of tubular work (mm)

Sy: yield strength (MPa).

17. A device for forming a tubular work into a shaped hollow product by using a hydroforming process, comprising:

a fixed female die having a longitudinally extending cavity, said cavity being sized to receive therein said tubular work;

a male die having a work surface, said male die being movably received in said female die in such a manner that the work surface of the male die faces said cavity to cause the cavity to be enclosed and have a polygonal cross section;

at least one projection formed on a lateral end of said work surface, said projection having a sloped surface angled relative to said work surface; and

an actuator which actuates said male die to press against said tubular work.

18. A device as claimed in claim 17, in which said cavity of said female die is defined by mutually facing vertical walls, a bottom horizontal wall and two slanted walls each extending between the vertical wall and the bottom horizontal wall.

19. A device as claimed in claim 17, further comprising: sealing tools which seal both open ends of said tubular work;

supporting members which stably support both end portions of said tubular work; and

feeding tubes which feed and draw a hydraulic fluid into and from an interior of said tubular work.

20. A device as claimed in claim 18, in which said cavity is formed, between each of the vertical walls and the corresponding slanted wall, with an axially extending stepped portion, the size of said stepped portion being smaller than the thickness of said tubular work and greater than one tenth of said thickness.

21. A device as claimed in claim 18, in which said cavity is formed with an extra slanted wall which extends between each of the vertical walls and the corresponding slanted wall, said extra slanted wall defining an angle relative to said vertical wall, said angle being within a range from 0° to 45°.

22. A device as claimed in claim 17, in which said cavity of said female die comprises mutually facing vertical wall, and in which said male die comprises two male die members which are movably received in said cavity, said two male die members being moved toward and away from each other by said actuator, each male die member having a work surface that directly contacts an outer surface of said tubular work upon pressing against said tubular work, the work surfaces of the two male die members being provided with said projections respectively.

23. A device as claimed in claim 22, in which each of the work surfaces of the two die male members is provided at lateral ends thereof with respective projections, each projection having a sloped surface which is exposed to said cavity and angled relative to the corresponding work surface.

24. A device as claimed in claim 23, in which the angle defined between said sloped surface and the vertical wall of the cavity is within a range from about 135° to about 165°.

25. A device as claimed in claim 24, in which the size and shape of said sloped surface of each projection are determined to satisfy the following equations:

$$4 \leq L/t_0 \leq 7.5$$

$$\alpha \geq 10 \times (L/t_0) + 68$$

wherein:

L: length of the sloped surface

t<sub>0</sub>: initial thickness of the tubular work

α: angle between the sloped surface and the vertical wall. 15

26. A device as claimed in claim 17, in which said female die includes four longitudinally extending concave surfaces which face said cavity, in which said male dies includes four male die members which are movably received in respective slots formed in said female die, in which each slot is exposed to the cavity at longitudinally extending ridges that constitute circumferentially terminal ends of the corresponding concave surfaces, and in which an imaginary straight line that passes through neighboring two of said ridges extends outside of said cavity. 25

27. A device for forming a tubular work into a shaped hollow product by using a hydroforming process, comprising:

a fixed female die having a longitudinally extending cavity, said cavity being sized to receive therein said tubular work and defined by mutually facing vertical walls, a bottom wall and two slanted walls each extending between the bottom wall of the corresponding vertical wall; 30

a male die having a work surface, said male die being movably received in said female die in such a manner that the work surface of the male die faces said cavity thereby to cause the cavity to be enclosed and have a polygonal cross section; 35

at least one projection formed on a lateral end of said work surface, said projection having a sloped surface which is angled relative to said work surface.

28. A device for forming a tubular work into a shaped hollow product by using a hydroforming process, comprising:

a fixed female die having a longitudinally extending cavity, said cavity being sized to receive therein said tubular work and defined by mutually facing vertical walls;

two male dies movably received in said female die in such a manner that respective work surfaces thereof face each other in said cavity thereby to cause the cavity to be enclosed and have a polygonal cross section;

at least one projection formed on a lateral end of each of the work surfaces, said projection have a sloped surface which is angled relative to the corresponding work surface.

29. A device for forming a tubular work into a shaped product by using a hydroforming process, comprising:

a fixed female die having a longitudinally extending cavity, four longitudinally extending concave surfaces which define four rounded corner portions of said cavity and four slots which are merged with said cavity, each slot being exposed to said cavity at a longitudinally extending ridges that constitute circumferentially terminal ends of the corresponding concave surfaces; and

four male dies movably and respectively received in the four slots of the female dies in such a manner that respective work surfaces thereof face the cavity, wherein an imaginary straight line that passes through neighboring two of said ridges extends outside of said cavity.

30. A device as claimed in claim 29, in which the work surface of each male die is formed at lateral ends thereof with respective concave recesses.

\* \* \* \* \*